

E. WEINTRAUB.  
LEADING-IN CONDUCTOR.  
APPLICATION FILED MAY 14, 1912.

1,154,081.

Patented Sept. 21, 1915.

*Fig. 1.*



*Fig. 2.*



WITNESSES:

J. Earl Ryan.  
J. Ellis Green.

INVENTOR:

EZECHIEL WEINTRAUB,  
BY *Albert S. Davis*  
His ATTORNEY.

# UNITED STATES PATENT OFFICE.

EZECHIEL WEINTRAUB, OF LYNN, MASSACHUSETTS, ASSIGNOR TO GENERAL ELECTRIC COMPANY, A CORPORATION OF NEW YORK.

## LEADING-IN CONDUCTOR.

1,154,081.

Specification of Letters Patent. Patented Sept. 21, 1915.

Application filed May 14, 1912. Serial No. 697,192.

To all whom it may concern:

Be it known that I, EZECHIEL WEINTRAUB, a citizen of the United States, residing at Lynn, county of Essex, State of Massachusetts, have invented certain new and useful Improvements in Leading-In Conductors, of which the following is a specification.

The present invention comprises a novel metallic seal for evacuated containers, and it involves the use of the metals tungsten and molybdenum for this purpose.

In the accompanying drawings, Figure 1 illustrates my invention as applied to a mercury vapor lamp consisting of a magnesium boro-silicate; and Fig. 2 illustrates a modification in which the conductors are sealed into a special form of glass.

In order to make a good vacuum-tight or hermetic seal in glass containers it is necessary that the glass and the metal have approximately the same coefficient of expansion, that the glass should wet the metal and thirdly, that the metal should either not oxidize during the sealing in process or that the oxid should be harmless.

Among the metals which are at all common tungsten, W, and molybdenum, Mo, are the only ones that have a lower coefficient of expansion than platinum. This is connected with the fact that the higher the melting point the lower the coefficient of expansion. I have found that tungsten and molybdenum make a vacuum-tight seal in boro-silicate glasses having approximately the same coefficient of expansion, say, between 3 to  $5 \times 10^{-6}$  and exerting what may be called a "wetting" effect upon the metal. As an example of such a glass, I mention sodium-magnesium boro-silicate, known in the market as "low expansion glass" which has a coefficient of 3.5 to  $4.5 \times 10^{-6}$ . I have found that when these metals are sealed in this glass that a wetting action takes place which is equal if not superior to the wetting action of ordinary lead glass for platinum. I have also made the discovery that the oxid of tungsten which forms on the wire during the sealing process in no way impairs the quality of the seal. This result is surprising as up to the present in the case of the various alloy substitutes proposed to replace platinum in lead glass the formation of an oxid has always stood in the way of a good vacuum-tight seal. In order to seal tungsten or molybdenum into boro-silicate glass, the seal-

ing in temperature must be considerably higher as the melting point of the boro-silicate is much higher than that of lead glass, and hence the tendency of the wire to oxidize must be greatly increased. It has been found, however, that oxidation of tungsten or molybdenum does not impair the finished seal. Apparently the oxid dissolves in or combines with the glass.

Fig. 1 shows a mercury arc lamp in which an open quartz tube 1, containing mercury electrodes 2, 3, is supported within an outer tube or envelop 4. This envelop 4 consists of sodium-magnesium boro-silicate and into it are sealed leading-in conductors 5, 6 consisting of tungsten or molybdenum. Both the body of the boro-silicate and the seals are better suited to withstand temperature changes without cracking than the former lead glass envelops provided with platinum leading-in wires. For this reason new fields in the electrical industry are opened to the utilization of exhausted containers provided with leading-in conductors. As an illustration, I may refer to the quartz mercury lamp which may be advantageously provided with tungsten or molybdenum seals by joining the boro-silicate glass to the quartz by means of a zone of vitreous material in which the proportion of basic constituents of the glass gradually diminish when passing from the glass to the quartz. This construction is described more fully in my co-pending application, Serial Nos. 678,741 and 698,740, filed May 21, 1912.

Seals made with the use of tungsten and molybdenum described in this application are not only cheaper than seals heretofore employed for evacuated containers, but by their use the construction of this class of apparatus may be considerably simplified.

Rectifiers, incandescent lamps, Röntgen tubes, Geissler tubes and the like can now be made not only of the boro-silicate but of other glass such as the so-called "heat resisting glass" or quartz by using one or a few intermediate glasses between the boro-silicate glass and the glass constituting the main body of the container, these glasses having intermediate coefficients of expansion. In the case of "heat resisting glass" shown in Fig. 2, only one intermediate glass is required, and even this may be omitted in some cases. The glasses of intermediate coefficients of expansion are readily obtainable

in the market. Of course in the event that it should be desired to constitute the body of the container of lead glass the junctures between the boro-silicate and the lead glass may consist of three or more mixtures of lead glass and boro-silicate glass, the proportion of either ingredients in the mixtures decreasing as the juncture with the material constituting the other ingredients is approached.

I desire by the appended claims to include a molybdenum as well as tungsten seal for evacuated containers.

What I claim as new and desire to secure by Letters Patent of the United States, is,—

1. A container, at least one region of which consists of boro-silicate glass having a coefficient of expansion of about 3 to

$5 \times 10^{-6}$ , and a tungsten conductor sealed therein.

2. An evacuated container, one region at least of which consists of a magnesium boro-silicate, and a tungsten conductor sealed in said silicate.

3. The combination of a sodium-magnesium boro-silicate glass, having a coefficient of expansion of about 3.5 to  $4.5 \times 10^{-6}$  and a tungsten conductor sealed therein and adhering at its surface to said glass.

In witness whereof, I have hereunto set my hand this eleventh day of May, 1912.

EZECHIEL WEINTRAUB.

Witnesses:

JOHN A. McMANUS, Jr.,  
FRANK G. HATTIE.